

## UNITED STATES PATENT OFFICE

2,235,466

## ANTIKNOCK MOTOR FUEL

Adrianus Johannes van Peski, Nicolaas Max,  
 Johannes Andreas van Melsen and Pieter Lucas  
 Stedehouder, Amsterdam, Netherlands, assign-  
 ors to Shell Development Company, San Fran-  
 cisco, Calif., a corporation of Delaware

No Drawing. Application June 6, 1938, Serial No.  
 212,128. In the Netherlands June 15, 1937

1 Claim. (Cl. 44—9)

This invention relates to gasoline type motor fuels, i. e., motor fuels suitable for use in gasoline engines, and more particularly deals with gasoline type motor fuels of high antiknock properties containing metal organic knock suppressors.

As is well known, certain mineral oil-soluble metal organic compounds, such as tetraethyl lead, nickel and iron carbonyls, ethyl selenide, etc., have the property of suppressing detonation or knock in spark-ignition engines. These compounds are generally known as antiknock compounds. While some of them are highly effective, they are all subject to at least one or several serious disadvantages, such as extremely insufficient solubility in hydrocarbons, high toxicity, poor storage stability, corrosiveness to the engine, etc.

It is a purpose of this invention to provide a class of efficient knock suppressors comprising metal organic compounds which are substantially free from the above disadvantages or at least possess them to a very much smaller extent. It is another purpose to provide non-toxic antiknock compounds readily soluble in gasoline having efficiencies comparable to those of tetraethyl lead; and it is a further purpose to produce antiknock gasolines containing metal organic antiknock compounds which upon storage for several months do not substantially decompose and depreciate in antiknock value.

We have discovered that metal organic compounds belonging to a class of compounds similar to those described in U. S. Patent No. 2,023,372 but differing from the latter by greater solubility in gasoline and greater antiknock value, may have knock-suppressing properties equal to or even better than the most potent known antiknock compounds. Our knock-suppressors are non-toxic, reasonably stable in storage, and gasolines containing small amounts thereof, i. e., equal in antiknock value to about 3 cm.<sup>3</sup> tetraethyl lead per gallon of gasoline, do not corrode valves and valve seats, nor do they cause undue wear of moving engine parts.

Our knock-suppressors are compounds of a metal having an atomic number of 26 to 29 inclusive, i. e., a metal selected from the class consisting of iron, nickel, cobalt and copper, and an organic substance containing both nitrogen and oxygen based on the following structural formula or its equivalent:



$\text{R}_1$  and  $\text{R}_2$  are hydrogen or organic radicals and  $\text{R}_3$  is an organic radical selected from the group consisting of alkyl, aryl and aralkyl, which may or may not contain one substituent. The radicals  $\text{R}_1$ ,  $\text{R}_2$  and  $\text{R}_3$  should preferably not contain more than 6 carbon atoms in total. Moreover,  $\text{R}_2$  jointly with  $\text{R}_1$  may form a ring structure, if the joined radicals contain a sufficient number of carbon atoms to form at least a 4-carbon ring. Suitable substituents in hydrocarbon radicals  $\text{R}_1$  to  $\text{R}_3$  are all those which are capable of forming substantially stable compounds with hydrocarbons, such as halogen, —CN, —OH, —OR, —COR, —NH<sub>2</sub>, —NHR, —NR<sub>2</sub>, —SH, —SR, —COOR, etc., neutral and basic substituents being preferred to those which are strongly acidic, such as —COOH, —SO<sub>3</sub>H, etc.

As is well known, in compounds of the above formula the double bonds are capable of shifting their exact location within the molecule depending upon the surrounding conditions, thereby forming the enol or keto forms and amino or imino forms, respectively. Therefore the following structures are considered full equivalents of the above:



and



The metal compounds of our invention may be conceived as salts or complex compounds or both. It is believed that the metal is usually attached to the oxygen as follows:



where Me is a metal having an atomic number of 26 to 29, and  $n$  is the valence of the metal. It is, however, likely that in addition there are links of secondary valences between the metal and the nitrogen, giving the compounds the character of complex compounds.

Our knock suppressors may be prepared by reacting for instance oxymethylene acetaldehyde or oxymethylene acetone or homologues thereof, either in the free state or in the form of their alkali metal salts or their compounds with alcohols, such as ethers and acetals, with primary organic amines, such as mono alkyl amines, mono alkanol amines, alkylene diamines, aniline, chlor aniline, etc. When starting from alkali metal salts of the oxymethylene compounds, the amines should be applied in the form of their salts, e. g., the hydrochlorides, whilst when starting from

acetals of the oxymethylene compounds it is preferable to carry out the reaction in the presence of water. The resulting reaction products are purified by suitable methods and are then converted to the desired metal compound for instance by treating same with copper acetate while in solution of a suitable solvent, such as an alcohol having not more than 4 carbon atoms.

The anti-knock value of our compounds depends to some extent on their volatility and solubility in gasoline. In the absence of polar radicals, solubility increases and volatility decreases in general with increasing molecular weight of the organic component. If both  $R_1$  and  $R_2$  are hydrogen the solubility in gasoline of the metal compound may be quite low, but sufficient, so that the corresponding compounds of copper and the ferrous metals are useful as antiknock compounds. If  $R_1$  or  $R_2$  or both are organic radicals, metal compounds thereof may be miscible with gasoline in substantially all proportions. On the other hand, if the molecular weight of the organic compound exceeds about 300 then the volatility becomes low and under average carbureting conditions a portion of the metal compound may deposit in engine manifolds instead of being drawn into the combustion chambers of the engines.

Compounds which are sufficiently volatile to reach the combustion chamber of gasoline engines under average carburetion conditions without material deposition in the manifold are usually distillable without substantial decomposition under high vacuum i. e., a vacuum of about 0.1 mm. mercury or lower.

35 Some of our metallic organic compounds are normally liquid while others are normally solid. Certain of those which possess highest antiknock values, such as the copper compound of methyl  
40 amino methylene acetone, are normally solid. However, it appears that the normally solid compounds have certain disadvantages as against those which are normally liquid. For instance, the former have a greater tendency of forming  
45 deposits in engine manifolds under average carburetion conditions and also in general are less soluble in gasoline. We have found, that frequently mixtures may be normally liquid, which mixtures consist essentially of our normally solid  
50 and normally liquid compounds and may contain the normally solid components in substantial proportions. Such liquid mixtures are highly useful as they may combine all the advantages of the normally liquid compounds with the very high  
55 antiknock value of the normally solid compounds.

55 antiknock value of the following solid compounds.  
Solubilities of little soluble compounds may  
also be improved by the addition of mutual sol-  
vents, such as the lower alcohols, ketones, ethers,  
amines, etc., boiling preferably within gasoline  
60 boiling range.

If desired gasoline type motor fuels may be prepared consisting entirely or predominantly of neutral oxyhydrocarbons, such as ethers, ketones, or alcohols, particularly those with branched 65 carbon chains and boiling within gasoline boiling range, containing small amounts of our anti-knock compounds.

The amounts of our antiknock compounds normally incorporated into the fuels to effect an improvement in the knock rating may vary from a bare trace to about .5% metal by weight of the fuel, although larger amounts may be used, if desired.

Of the four metals iron, nickel, cobalt and copper, found to possess the high antiknock proper-

ties when combined with the organic components described, copper and cobalt are the most outstanding and effective.

We have further found that the copper or cobalt compounds of alkyl and alkylene amino methylene ketones and of alkyl and alkylene amino methylene aldehydes, in which the alkyl or alkylene radicals preferably contain not more than 6 carbon atoms, are especially powerful knock suppressors. Cupric or cobalt methyl amino methylene acetone has the formula: 5 10



Other suitable compounds are: the cupric or cobalt compound of allyl amino methylene pinacoline having the formula: 20



the cupric or cobalt compound of ethyl amino methylene acetaldehyde.



Further examples of suitable compounds are 40 the copper, iron, nickel or cobalt compounds of the following organic compounets:



Also mixed compounds of copper or the ferrous metals with different species of the organic components hereinbefore described, or with other compounds, such as alcohols, phenols, mercaptans may be employed. For instance the basic alcoholate of the cupric compound of methyl amino methylene pinacoline was found to be an active antiknock compound. It may be represented by the formula:



Furthermore mixtures of two or more of our anti-knock compounds, as well as mixtures with other anti-knock compounds, such as tetraethyl lead, may often be used to great advantage.

5 The following illustrative examples further demonstrate our invention:

*Example I*

To two samples of a gasoline, having an octane number of 40, the copper compound of methyl aminomethylene acetone was added in quantities, so that the blended gasoline contained .05% and .1%, respectively copper by weight of the gasoline. As a result the octane numbers were raised 15 to 59 and 69 respectively.

The same gasoline was blended with tetraethyl lead in quantities to produce two blends containing .05% and .1% lead by weight of the gasoline. The resulting octane numbers were 55 and 66 20 respectively.

*Example II*

To the gasoline of Example I .05% by weight of copper was added in the form of the copper compound of methyl aminomethylene 2-pentanone. The octane number rose to 58.

*Example III*

.1% copper in the form of the copper compound of ethyl aminomethylene acetone was 30 added to the gasoline of Example I, thereby raising its octane number to 67.

*Example IV*

.1% by weight of copper in the form of the cupric compound of allyl aminomethylene acetone raised the octane number of a gasoline from 35 40 to 69.

*Example V*

To a gasoline, the octane number of which 40 was 40, .04% by weight of cobalt was added in the form of the cobaltous compound of ethyl aminomethylene acetone. The octane number rose to 64.

*Example VI*

To a mixture of 90% iso-octane and 10% normal heptane, having an octane number of 90, .1% of copper in the form of cupric ethyl aminomethylene acetone was added whereby the octane 50 number was raised to 99.5.

*Example VII*

.08% copper in the form of cupric beta oxyethyl aminomethylene acetone



raised the octane number of a gasoline from 40 to 52.5.

*Example VIII*

.10% copper in the form of cupric ethyl aminomethylene acetaldehyde



raised the octane number of a gasoline from 40 to 64.5.

*Example IX*

.03% copper in the form of a normally liquid mixture consisting of 30 parts by weight solid cupric methyl aminomethylene acetone and 70 parts of liquid cupric ethyl aminomethylene acetone raised the octane number of a strongly aromatic gasoline from 78 to 86.

5

10

.1% copper in the form of cupric ethyl aminomethylene acetone in a mixture of 20% of this compound and 80% aniline raised the antiknock value of a gasoline from 40 to 71.

15

*Example X*

.1% cobalt in the form of the cobaltous compound of ethyl aminomethylene acetone raised the octane number of a hydrogenation gasoline (prepared from Venezuelan gasoil) from 79 to 97.

20

*Example XI*

.1% nickel in the form of the nickel compound of ethyl aminomethylene pinacoline raised the octane number of a gasoline from 40 to 60.5.

25

*Example XII*

.1% cobalt in the form of the cobaltomethylate of ethyl aminomethylene acetone

30



when added to a gasoline with an octane number of 40 raised this number to 61.

35

*Example XIII*

.1% copper in the form of the cupric compound of beta ethoxyethylamino methylene acetone

40



raised the octane number of a gasoline from 40 to 61.

45

*Example XIV*

.1% copper in the form of the cupric compound of beta ethoxyethylamino methylene acetone

40

raised the octane number of a gasoline from 40 to 60.

50

*Example XV*

.05% cobalt in the form of the cobaltous compound of ethyl aminomethylene acetaldehyde raised the octane number of a gasoline from 40 to 60.

55

We claim as our invention:

An improved motor fuel, which comprises a gasoline type motor fuel and a small amount of a normally liquid mixture consisting of the normally solid cupric methyl amino methylene acetone and of the normally liquid cupric ethyl amino methylene acetone.

55

ADRIANUS JOHANNES VAN PESKI.  
NICOLAAS MAX.

JOHANNES ANDREAS VAN MELSEN.  
PIETER LUCAS STEDEHOUDER.

60